

Jan. 20, 1931.

C. KANNEL

1,789,629

METHOD OF TANNING SOLE LEATHER

Filed April 4, 1928

*Fig. 1,*



*Fig. 2,*



INVENTOR  
*Charles Kannel*  
BY  
*Mary. Grumman* ATTORNEY

## UNITED STATES PATENT OFFICE

CHARLES KANNEL, OF BROOKLYN, NEW YORK

## METHOD OF TANNING SOLE LEATHER

Application filed April 4, 1928. Serial No. 267,153.

The present invention relates to a method of tanning leather.

It is already well known to tan leather in a vacuum as for instance according to the method of Nance of France. But, the performance of the Nance method requires the building of relatively large stationary vessels made of copper, brass or concrete which must be equipped with heating means and means for supplying compressed air. According to the Nance method it takes considerable time to complete the tanning.

The object of my invention is to simplify the method so that comparatively simple means can be used for carrying out the method and whereby the latter can be completed in the shortest possible time. My new process consists in that the raw skins are first limed, for a short period of time, then on removal of the hair and flesh are cleaned, then, without, as hitherto, first decalcifying, are placed into a bath composed of about 100 quarts of water, 250 grams of potassium chromate, 200 grams boracic acid, 250 grams sulphuric acid or similarly acting acids, such as 180 grams of formic or 210 grams of butyric acid, to which may be added about 50 grams of glycerine. In this bath the skins are kept for about 16 to 24 hours.

By treatment in such bath the skins are rendered insensitive against the highly concentrated tanning substances to be used in the process and on the other hand receptive of said substances.

On the removal of said skins from said bath, they are placed in a suitably reinforced drum containing any kind of tanning solution of 12°-14° Baumé. During the treatment of the skins in said drum the latter is maintained in motion and under the action of suction, the air therein rarified and the injurious gases produced during the tanning process and which render the leather brittle are withdrawn.

By my new method the tanning process can be completed in a period of less than 24 hours and the product derived therefrom is of the best quality, such as produced by the hitherto used very complicated processes.

Apart from that, there is a great saving

of tanning substance, which through long lasting treatments are lost owing to the carbonic acid formed.

A great advantage of my method is that any available tanning vessel can be employed for carrying out the same.

To make my invention more clear I have illustrated the same in the accompanying drawing in which similar reference characters denote corresponding parts and in which Fig. 1 is a longitudinal section of a common wooden barrel with the means for evacuating the same and Fig. 2 is a cross section of a slightly modified construction.

In the drawing according to Fig. 1 an ordinary wooden or wood lined suitably reinforced barrel 10 is mounted on a longitudinally perforated shaft 11 which is revolved from a suitable source of power through belt and pulley 12, 13 respectively. The shaft is rotatively supported in a suitable frame 14 and one end thereof is connected to a vacuum pump 16 by a hose or pipe 16 by means of a suitable joint 16' so that said shaft 11 may be rotated while connected to said pump.

In Fig. 2 the shaft 11 of the barrel 10 is adapted to receive oscillatory motion. To this end the shaft may be provided at its outer ends with gears 17 each having a few teeth 18 which when the shaft is rotated, will alternately mesh with parallel stationary racks 19, 20 that according to the present example are shown to be integral parts of the frame.

The movement imparted to the vessel either rotary or oscillatory expedites the tanning process in that the friction caused between the pieces of leather or hides contained in the vessel produce the heat necessary for the process and which causes the opening of the pores in said material so that the tanning substances can effectively pass into the material.

What I claim is:—

1. In a process of tanning sole leather or the like the step of treating the same in a rotating condition in a tanning substance under a constantly maintained vacuum.
2. A method of tanning sole leather con-

95

100

sting in treating limed cleaned skins in a bath to which potassium chromate has been added and then in a rotating condition in a tanning substance under a constantly maintained vacuum.

3. In the process of tanning leather rapidly comprising the step of treating the limed skins in a bath to which potassium chromate, boracic acid, another non-oxidizing acid, and glycerine, have been added.

4. A method of tanning leather including the steps of placing the limed cleaned skins in a bath to which potassium chromate, boracic acid, another non-oxidizing acid and glycerine have been added, then treating them in a rotating condition drum containing a tanning solution, agitating said skins therein and at the same time continuously maintaining a vacuum for withdrawing the gases formed by the chemical reaction.

5. A method of tanning leather including the steps of pretreating the limed skins in a solution to which potassium chromate and glycerine have been added and then treating them in a tanning solution and a constantly maintained vacuum.

6. A method of tanning leather including the steps of pretreating the limed skins in an acid bath and then treating them in a tanning solution under a constantly maintained vacuum as they form.

7. In the process of tanning leather the step of pretreating the limed cleaned skins in a bath containing the reaction products of a mixture of potassium chromate, boracic acid, glycerine and sulphuric acid and water.

8. In the process of tanning leather, the steps of pretreating the limed cleaned skins for 16 to 24 hours in a bath containing the reaction products of a mixture of substantially 250 grams of potassium chromate, 200 grams of boracic acid, 250 grams of sulphuric acid and 50 grams of glycerine to every 100 quarts of water.

9. In the process of tanning leather the step of pretreating the cleaned limed skins for 16 to 24 hours in a bath to which substantially 250 grams of potassium chromate, 200 grams of boracic acid, 210 grams butyric acid and 50 grams of glycerine to substantially every 100 quarts of water have been added.

10. In the process of tanning leather the step of pretreating the cleaned limed skins for 16 to 24 hours in a bath to which substantially 250 grams of potassium chromate, 200 grams of boracic acid, 180 grams of formic acid and 50 grams of glycerine to substantially every 100 quarts of water have been added.

11. A method of tanning leather including the step of pretreating the cleaned limed skins in a bath to which potassium chromate, boracic acid, glycerine and another non-oxidizing acid have been added and then

subjecting said treated skins to a tanning solution for approximately 24 hours under a constantly maintained vacuum for withdrawing as formed the gases caused by the tanning reaction.

12. A bath for use in the process of tanning leather comprising the reaction products of a mixture of potassium chromate, boracic acid, sulphuric acid and glycerine in water.

13. A pretreating bath for use in the process of tanning leather comprising the reaction products of a mixture in the approximate proportions of 250 grams of potassium chromate, 200 grams of sulphuric acid and 50 grams of glycerine in every 100 quarts of water.

14. A bath for use in the process of tanning leather comprising a mixture of potassium chromate, boracic acid, an other non-oxidizing acid and glycerine in water.

15. A method of tanning leather including the steps of pretreating the limed skins in an acid bath and then treating them in a rotating condition in a tanning solution and continuously maintaining a vacuum for withdrawing the gases formed by the chemical reaction as they form.

16. A bath for use in the process of tanning leather comprising the reaction products of a mixture of potassium chromate, boracic acid, butyric acid and glycerine in water.

17. A bath for use in the process of tanning leather comprising the reaction products of a mixture of potassium chromate, boracic acid, formic acid and glycerine in water.

In testimony whereof I affix my signature.

CHARLES KANNEL.

105

110

115

120

125

130